

May 2, 1933.

A. C. FISCHER

1,907,417

SURFACING UNIT

Filed July 9, 1928

Fig. 1



Fig. 2



Fig. 3



Fig. 4



Fig. 5



Inventor:  
Albert C. Fischer,  
By *Albert C. Fischer* atty.

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## SURFACING UNIT

Application filed July 9, 1928. Serial No. 291,326.

This invention relates to surfacing units, and aims to provide novel and improved slabs adapted to be anchored to a surface to be covered for forming a waterproof and acid-proof layer.

The invention consists in the features, combinations and arrangements, hereinafter described or claimed, for carrying out the above stated object and such other objects as will 10 hereinafter appear.

Generally described the invention comprises units preformed from a homogeneous mixture of bituminous material, linear fibers, and mineral material. The mixture is prepared and then formed into a standard sheet, from which the units may subsequently be shaped to conform to the surface to be covered. Means are provided on the units for embedding within a plastic layer to secure 20 them in place and prevent any loosening thereof which would allow access of water and other deleterious matter to the protected understructure.

In the drawing:—

25 Figure 1 is a perspective view of a unit embodying my invention;

Figure 2 is a perspective view of a modified embodiment;

30 Figure 3 is a perspective view of a conduit lined with the novel units;

Figure 4 is a sectional view of a wall structure faced with the novel units;

Figure 5 is a perspective view of a modified manner of attaching the units.

35 Specifically described the invention is typified by unit 2 preformed from a homogeneous mixture of bituminous compound, filling and hardening material. The bituminous material is preferably prepared from blown and hard asphalt, grahamite and others, or one that has been blown to a very high melting point and has considerable binding qualities. In preparing a suitable mixture the proportion of bituminous compound to the

40 filling and hardening material may be modified, depending upon the use to which the slabs are to be put. One example of a suitable mixture comprises bituminous compound between forty and fifty per cent (40-50%), linear fiber between ten and twenty

per cent (10-20%) and earthy material aggregating about forty or fifty per cent (40 or 50 per cent). The fiber is preferably composed of felt fiber, but may be digested or undigested straw, flax, hemp or any soft 55 fibrous material. If desired the fibrous material may be reenforced with tougher fiber, The mineral filling is represented by such materials as limestone dust, slate dust, bentonite, barytes, powdered silica, terra cotta 60 dust, asbestos float, asbestos sand or may be composed of short asbestos fiber or asbestos fiber waste, or asbestos waste combined with magnesia, or other cement ground up into small particles. Sheets formed from this material may be easily arched as indicated by 3 to conform to the curvature of any conduit 4, in which they are employed to line any part or all of the conduit.

Where the sheets are not to be arched, they 70 are preferably made more dense and rigid by employing the harder bituminous material and a greater proportion of mineral material. For example, a harder unit may be formed from a mixture comprising approximately 75 sixty to seventy per cent (60-70%) mineral matter and thirty to forty per cent (30-40%) of the harder asphalt. The more dense units are suitable for wall facing, flooring, paving, or the like, and may be secured 80 to a monolithic plastic foundation 5.

The units may be advantageously provided with projections 6 so that a secure attachment can be made to any plastic layer in which they are embedded. Such a union 85 firmly anchors the units and prevents any displacement which would impair the protecting layer. A tight joint is obtained between adjacently laid units by forming mating tongues 7 and grooves 8 on the edges.

90 It will be seen that units formed from the materials above enumerated may be made of a standard size and then subsequently shaped to conform to the surface on which they are to be laid, whereas if constructed of tile, cement or the like, they would have to be of 95 separate sizes for each particular piece of work. These are secured directly to the conduit or by means of a thin layer 9 of cement or other adhesive.

In Figure 5 an alternative securing means is illustrated for joining the units into a covering, the same comprising band 10 inserted through individual units laid side by side in rows with broken joints.

Obviously the invention is not limited to the details of the illustrated modifications, all of which may be variously modified. Moreover, it is not indispensable that all features of the invention be used conjointly as certain of them may be employed to advantage in various different combinations and sub-combinations.

Having described my invention, I claim:

15 1. Lining units for conduits comprising a homogeneous body of yieldable fiberized bituminous material arched to conform to the conduit to be lined, and projections on the face of the unit for keying same to the conduit.

20 2. Lining units for conduits comprising a homogeneous body of yieldable fiberized bituminous material arched to conform to the conduit to be lined, projections on the face 25 of the units for keying same to the conduit, and the edges tongued and grooved to match with adjacently laid units.

30 3. Protecting units for curved surfaces, comprising a homogeneous mixture of yieldable fiberized bituminous material arched to conform to the contour of the surface to be covered, anchoring keys on one face of the unit, and rounded tongue and grooved edges whereby the units may be laid adjacently 35 with tight joints.

40 4. Lining units for conduits comprising a preformed body of fiberized bituminous composition of yieldable character whereby same may be arched to conform to the contour of the conduit to be lined, and means for attaching the lining in position.

45 5. Lining units for conduits comprising a preformed body of fiberized bituminous composition of yieldable character provided with matched edges whereby adjacent units may be closely fitted in any angular position, and means for attaching the lining in position.

Signed at Chicago, in the county of Cook and State of Illinois, this 30th day of June 50 1928.

ALBERT C. FISCHER.